

# UNITED STATES PATENT OFFICE.

FRIEDRICH LEHNER, OF ZURICH, SWITZERLAND.

## MANUFACTURE OF ARTIFICIAL HEMP FIBER.

No. 853,098.

Specification of Letters Patent.

Patented May 7, 1907.

Application filed May 16, 1906. Serial No. 317,240.

*To all whom it may concern:*

Be it known that I, FRIEDRICH LEHNER, a citizen of Germany, residing at Zurich, Switzerland, have invented certain new and useful Improvements in the Manufacture of Artificial Hemp Fiber; and I do hereby declare the following to be a full, clear, and exact description of the invention, such as will enable others skilled in the art to which it applies to make and use the same.

This invention relates to an improved method of manufacturing artificial hemp fiber having for its object the provision of a substitute material which, while possessing the characteristic appearance and advantages of the natural product, is without the disadvantages accompanying the same.

Natural unshackled hemp fiber freed from woody matter and in lengths of about a half meter, finds extensive employment in the industries and especially in the manufacture of hats. This material is inconvenient in use, however, by reason of the difficulties encountered in working the same, due to the troublesome knitting together of the single strands in producing small threads or ribbons as a work material. The strands or filaments manifest a very undesirable lack of uniformity in thickness and breadth, due in part to the preparation of the same from the plant and, moreover, the many irregularities and knots are troublesome obstacles to the satisfactory working of the same in the arts. On the other hand, the natural hemp fiber has a characteristic dull luster which is liked in the art and which is not possessed by the substitutes which have been proposed hitherto.

By this invention it is proposed to produce an article possessing every appearance of the natural hemp fiber without its disadvantages, and available for use in unlimited lengths and of a uniform thickness and width.

It has already been proposed to form textile work material by gluing together, according to the size required, of one or more filaments or strands lying parallel to each other. A thread so formed, however, corresponds in appearance to the material from which it is made. A thread made from silk, for instance, shows a characteristic natural silk gloss, artificial silk has a more highly lustrous strawy appearance, and that formed from bleached cotton shows the duller white tone of the raw material. None of these materials have been made to show the char-

acteristic dull gloss and peculiar color of the hemp fiber, nor do they possess its capacity for dyes.

By the improved process herein set out, lustrous threads of silk, artificial silk, mercerized cotton and the like, either singly or in combination with two or more similar threads, are subjected to a process by which their luster is dulled, by the same means or at the same time that they are glued together to form a thread or ribbon, corresponding to that of the hemp fibers desired to be produced.

According to this process, one or more lustrous filaments of natural silk, artificial silk, viscose silk, mercerized cotton and the like, are subjected to a bath in a suitable binding material insoluble in water, such, for instance, as collodion, dissolved cellulose or viscose. After removing the surplus binding material, that remaining is fixed in a known manner by drying or by decomposition, as by subjecting to an acid, whereupon the thread or ribbon so obtained is wound upon a reel or spool for future use.

For the purpose of dulling the luster of the material to correspond to that which it is to simulate, to the binding material, either before, during, or after the manufacture of the ribbon, a suitable luster-dulling coating substance is added, such, for instance, as heavy spar, pulverized chalk, zinc white, amorphous sulfur and the like, and also an appropriate dye to produce the yellowish shade characteristic of the hemp fiber. It is also possible, however, to produce this coating or luster-modifying effect by a chemical treatment of the binding material itself, either by a separate process or simultaneously with the fixing of the same, as, for instance, where a watery viscose solution is used, the treated ribbon or thread, before the binding material has become fixed, can be drawn through, or otherwise subjected to a mineral acid, by which treatment sulfur is separated out. This separated amorphous sulfur suffices for the coating and dulling of the thread or ribbon so that a further addition of coating material to the binding material for that purpose is not necessary.

Having thus fully described my invention, what I desire to secure by Letters Patent of the United States, is:—

1. The process of producing artificial hemp fiber which consists in gluing together a plurality of lustrous filaments with a binder con-

taining a coating material adapted to dull the luster of the product.

2. The process of producing artificial hemp fiber which consists in gluing together a plurality of lustrous filaments and modifying the luster of the same to approximate that of hemp fiber.

3. The process of producing artificial hemp fiber which consists in gluing together a plurality of lustrous filaments by a viscose solution, and subjecting the freshly treated fibers to a mineral acid, whereby the binding material is fixed and the luster of the product is dulled.

4. The process of producing artificial hemp fiber which consists in gluing together a plurality of lustrous filaments by a viscose solution containing a suitable dye, and subjecting the freshly treated filaments to the action of a mineral acid, whereby the binding material is fixed and the amorphous sulfur is separated out to dull the luster of the product.

In testimony whereof I hereunto affix my signature in the presence of two witnesses.

FRIEDRICH LEHNER.

Witnesses:

A. LIEBERKNECHT,  
WALKER RASCHERT.